

## UNITED STATES PATENT OFFICE

2,363,947

## ALLOYS FOR CUTTING TOOLS

Anthony G. de Golyer, Old Greenwich, Conn.,  
assignor to Laurence A. Janney, Stamford,  
Conn., as trustee

No Drawing. Application March 11, 1943,  
Serial No. 478,828

7 Claims. (Cl. 75—123)

This invention contributes a new and useful alloy especially valuable in metal-cutting tools and other implements that require similar properties. An alloy embodying the invention has novel and distinctive qualities of hardness, strength, stability in fabrication and use at high temperatures, and exceptional efficiency when applied to metal cutting and working.

An illustrative embodiment, herein called for brevity "Alloy A" comprises the following constituents, in the proportions indicated, which were ascertained by analysis of the cast product:

|            | Per cent                                                        |
|------------|-----------------------------------------------------------------|
| Tungsten   | 15.80                                                           |
| Molybdenum | 3.90                                                            |
| Vanadium   | 0.90                                                            |
| Cobalt     | 29.70                                                           |
| Carbon     | 0.67                                                            |
| Boron      | 0.70                                                            |
| Iron       | the balance excepting minor amounts<br>of manganese and silicon |

The specific alloy A when molten is preferably cast centrifugally. The cast forms have a hardness of about 60 to 65 Rockwell C. An illustrative method of treating the castings is as follows: They are annealed at a temperature range of 1600° F. to 1800° F. One specific procedure is to hold the castings at about 1650° F. for two or three hours and allow them to cool slowly to a temperature somewhat below 1200° F. When so annealed they show approximately 46 Rockwell C. and are in condition to be ground or machined.

If alloy A is to be used in cutting tools or the like, a preferred hardening procedure is as follows: The castings are preheated at about 1100° F. for about half an hour, and then introduced to a second preheating at 1500° F. to 1550° F. and held at such temperature long enough for thorough heating. They are then transferred to a furnace in which the temperature is from 2150° F. to 2175° F. When the entire body of metal has reached the high temperature the castings are quenched in oil. At this stage they show about 62 Rockwell C.

The quenched castings are cooled to about 200° F. to 300° F. when they are ready for drawing. Multiple drawings are desirable, especially for the purpose of stabilizing the ultimate hardness of the castings as presently described. Castings of small or moderate size are drawn first for about one hour at 900° F. For larger pieces a longer drawing period is usually desirable. After this first drawing, the castings are permitted to cool slowly to room temperature. Thereafter they are

drawn a second time at from about 1150° F. to 1375° F. according to the ultimate degree of hardness desired. The duration of the second draw is regulated according to the size of the individual castings, in the range of forty-five minutes to two hours for the usual range of sizes. For some purposes a single draw, to the higher temperatures, may suffice; but when cutting tools are the object the multiple drawings, approximately as above described, are preferable because they improve the distinctive characteristics of the alloy.

Following the illustrative method, the alloy A castings exhibit a combination of properties that are especially valuable in metal-working tools and the like. In such use, the alloy is strikingly superior in numerous respects to the best of the previously known products it is intended to supersede. For instance, the alloy is highly responsive to thermal treatment by which any desired degree of hardness within the Rockwell C. range of 60 to 72 may be developed, controlled and maintained with remarkable precision. Such predetermined hardness is retained with great stability at high temperatures as (a) in reheating for brazing or welding by which tool shanks are equipped with cutting tips made from the new alloy; and (b) in conditions calling for unusually high red hardness as when cutting metal at temperatures between about 1000° F. and 1250° F. The alloy is highly resistant to abrasive wear at temperatures up to about 1250° F., and to shock and compression.

An outstanding characteristic of alloy A when treated as described, is its extraordinary stability, already mentioned, against permanent softening or other deterioration when reheated at temperatures up to 1250° F. or 1275° F., even for considerable durations, as for a time long enough for perfecting a brazed or welded joint. Such stability makes it possible to apply the alloy in the form of tool tips by the generally advantageous furnace brazing, for example, with minimum if any danger of impairing the pre-developed hardness of the alloy tip.

It is noteworthy that the maximum drawing temperature can be placed at or somewhat above the temperature expected to be generated on reheating, as in a metal-cutting or similar operation. When that is done the properties of the alloy are stabilized so that reheating to any temperature at or below the maximum drawing temperature causes little or no deterioration or loss of operating efficiency. Along with this important inherent stability, the alloy has adequate

plasticity and mechanical strength in maximum ranges of working temperatures, sufficient to supply uncommonly long tool life under severe operating conditions. Those qualities persist throughout the wide range of secondary hardnesses, between about 60 and 70 Rockwell C, any degree of which may be selectively predetermined with surprising accuracy due to the reliable responsiveness of the alloy to the designated character of thermal treatment.

I have demonstrated that the above-described properties and characteristics of alloy A will inhere effectually, though with some absolute and relative variations in degree, in alloys composed of these ingredients within the approximate ranges stated as follows: tungsten 12.00% to 20.00%; molybdenum 1.00% to 6.00%; cobalt 20.00% to 35%; boron 0.45% to 0.95%; carbon 0.35% to 0.85%; and the remainder principally iron, in a percentage exceeding that of the percentage of cobalt in any specific composition. The respective properties and characteristics of alloys formed within these ranges, corresponding to those of alloy A, can be developed, controlled and maintained by thermal treatment of the character I have disclosed.

It will be noted that alloy A contains a small percentage of vanadium. Vanadium, however, is not an essential component, though small amounts of it may have some beneficial influence in limiting the grain-size of constituents of the alloy, especially after thermal treatment. Though the vanadium appears to have little if any direct effect upon the novel major properties of the alloy, it is feasible to add it in the range of approximately 0.20% to 3.00% as an auxiliary alloy element.

Small amounts of manganese and silicon may be present as incident to manufacture, for their usual purposes of aiding deoxidation during the production of the alloy, and they are commonly present in scrap or ferro alloys. The content of manganese and silicon should not exceed about 0.70% and 0.90%, respectively, and it is considered advisable to limit the manganese to about 0.30% and the silicon to about 0.50%. When phosphorus and sulphur are present as incidental impurities, they should be limited to about 0.030% phosphorus and 0.010% sulphur.

The valuable inherent properties that characterize the new alloy result from the novel composition of elements, within the respective ratios specified herein. I intend, therefore, to restrict the amounts of any other elements which may be present, from any cause, to percentages which are substantially ineffectual on the valuable properties, as well as on the chemical and physical reactions which take place within the alloy at different stages of production of forms intended for industrial use. For example, chromium has been long considered an essential alloy element in high speed steels and other cutting alloys which are hardened by thermal treatment, as well as in cutting tool alloys which are not responsive to thermal treatment.

I have discovered that when chromium, even in quite small amounts, is present in the new alloy its mainly important properties are adversely affected. As an illustration, when 1% or less of chromium is present the responsiveness of the alloy to heat treatment is altered to such an extent that a precise degree of hardness can not be developed, and the alloy can not be adequately stabilized against subsequent variation of hardness when heated to temperatures from 1,000°

F. to 1,300° F. As a further illustration, when the amount of chromium present is in the range from 2% to 4% the degree of red hardness is materially reduced and the general metal cutting efficiency is greatly inferior to that of the alloy which is substantially free from chromium. The adverse effects of chromium are shown by the comparative figures for alloys A and B in Table II. Therefore, the new alloy should be substantially free from chromium.

To exemplify the distinctiveness of the new alloy and technique, the following discussion and tables are presented, based upon comparative demonstrations of three alloys, that were composed as follows:

- A. The alloy A already identified above.
- B. A test alloy of like composition with the addition of 4.00% chromium.
- C. A specimen of commercial standard 19-4-2 high speed steel with 12.00% cobalt.

The percentages given were ascertained by chemical analysis of the three alloys.

Table I

|            | A                                                                              | B        | C        |
|------------|--------------------------------------------------------------------------------|----------|----------|
|            | Per cent                                                                       | Per cent | Per cent |
| Tungsten   | 15.80                                                                          | 15.40    | 18.90    |
| Molybdenum | 3.90                                                                           | 3.70     | 0.85     |
| Chromium   | None                                                                           | 4.20     | 3.96     |
| Vanadium   | 0.90                                                                           | 1.20     | 1.92     |
| Cobalt     | 29.70                                                                          | 29.20    | 12.40    |
| Carbon     | 0.67                                                                           | 0.71     | 0.81     |
| Boron      | 0.70                                                                           | 0.72     | None     |
| Iron       |                                                                                |          |          |
|            | Balance in each composition except for minor amounts of manganese and silicon. |          |          |

Specimens of alloys A and B were heated for quenching according to the method disclosed above. Specimens of steel C were quenched in oil (125° F.) from 2425° F., as recommended by the producer for development of maximum hardness of this steel. Separate specimens of the respective samples were used for each of a series of drawing temperatures. All specimens were carefully ground to remove any decarburized material before hardness determinations.

After drawing alloys A and B and steel C for one hour, except as indicated below, the Rockwell C scale hardness values were ascertained as follows:

Table II

|                      | Temperature | A  | B  | C  |
|----------------------|-------------|----|----|----|
| Quenched             |             | 62 | 64 | 63 |
| 800° F.              |             | 63 | 62 | 62 |
| 900° F.              |             | 65 | 63 | 64 |
| 1,000° F.            |             | 67 | 64 | 65 |
| 1,050° F.            |             | 68 | 64 | 65 |
| 1,100° F.            |             | 70 | 65 | 65 |
| 1,150° F.            |             | 71 | 63 | 62 |
| 1,200° F.            |             | 70 | 60 | 60 |
| 1,250° F.            |             | 68 | 58 | 58 |
| 1,300° F.            |             | 65 | 54 | 54 |
| 1,350° F.            |             | 62 | 51 | 49 |
| 1,400° F. (30 mins.) |             | 61 | 50 | 43 |

<sup>1</sup> Deep scaling and decarburization required heavy grinding to provide solid metal; highest reading is given.

Several specimens of each of the A, B and C compositions, were drawn respectively to average hardness of 64 to 65 Rockwell C, and were brazed with silver solder to shanks  $\frac{3}{4}$ " x  $1\frac{1}{2}$ " x 7", and  $1\frac{1}{4}$ " x  $2\frac{1}{2}$ " x 14". Standard practice was followed in all cases. The brazing temperature was between 1300° F. and 1350° F. All of the B and C tips had their hardness decreased, by the heat, from 3 to 5 Rockwell C points. The tips of alloy A showed no deterioration in hardness or

otherwise. Equivalent results were obtained from like specimens when they were torch-brazed by a commercial tool-maker.

Four specimens of alloys A and B and steel C were quenched, as indicated above, and after cooling to approximately 250° F., were drawn at 800° F. for one hour and allowed to cool in still air to room temperature. The three sets of specimens were subsequently drawn and cooled from each of the successive temperatures indicated in Table II, to and including 1350° F. Hardness determinations after each drawing and cooling did not show any measurable difference from the figures in Table II, except in the case of steel C, the specimens of which had an average Rockwell C hardness of 56, 52 and 48 after drawing at 1250°, 1300° and 1350° F., respectively.

It will be apparent from Table II that; (a) an appreciably higher hardness is developed in alloy A than in either of the other materials; (b) that the upper limit of maximum hardness for alloy B and steel C is 1100° F., while the maximum hardness of alloy A persists from 1100° F. to 1200° F., which is considered to be the upper red-hardness temperature range to which metal cutting-tools are subjected under more or less severe operating conditions; (c) when alloy B and steel C are heated for one hour at 1150° F. the hardness of each is permanently reduced to the minimum degree at which a tool will cut steel with efficiency under favorable conditions, whereas, the hardness of alloy A is not lowered to 62 Rockwell C until after the material has been heated at 1350° F. for one hour.

This comparison demonstrates a substantial and important distinctiveness in the chemical and physical reactions which occur as a result of drawing alloy A as compared with those which take place in the other two compositions when drawn within the same temperature range, i. e., 800° F. to 1350° F. It is especially noteworthy that alloy A is conspicuously more resistant to appreciable and rapid loss of hardness at temperatures materially in excess of that at which maximum secondary hardness is attained.

I have found that when any desired degree of hardness (within feasible ranges above indicated) is developed in the present alloy by drawing to temperatures at and higher than that required for development of maximum secondary hardness, the alloy is remarkably stabilized against measurable variation of such developed hardness through diffusion or atomic rearrangement when subsequently reheated, in use or from treatment, to any temperature up to that at which the desired degree of hardness was developed.

I have also found that the above-described drawing procedure produces an unusually high degree of red-hardness, i. e., when a desired degree of hardness has been attained in the manner just illustrated, the present alloy retains an exceptionally high percentage of such hardness at temperatures generated in a tool during metal cutting operations.

As indicated in the first two columns of Table II, each temperature in the drawing range produced a corresponding high degree of hardness in alloy A. Such respective degrees of hardness may be reproduced selectively with reliable precision in the practice of this invention, so as to predetermine a desired hardness for any of my new compositions, within the percentage ranges above defined, embodying the general characteristics of alloy A.

Specimens of a chosen specific form of the

new alloy, treated, as already disclosed, through the first drawing step, may then be heated to progressively increased temperatures in the second drawing, and the Rockwell C hardness at each such temperature may be observed. Thereafter, if the same specific alloy is drawn to any said temperature, it will have in practically adequate and dependable approximation the same corresponding hardness under equivalent conditions as in the specimens first drawn. That is, as exemplified in Table II, the tested samples of alloy A acquired hardness of 65 points at 1300° F.; and it is safely predictable that in all instances, under like conditions and preliminary treatment, any specimen of alloy A can be given the same hardness (within permissible tolerances) by drawing it to the same temperature.

And when the drawing treatment has been carried to a given temperature to produce a corresponding predetermined hardness, the alloy will retain that hardness with unique stability when reheated to any temperature at or below the maximum drawing temperature used. Thus, this invention provides a novel alloy of peculiar responsiveness to thermal treatment, and an accurately regulable character of thermal technique, such that any example of such alloy can be hardened to any selected degree within an exceptionally wide range, and then reheated to substantially the maximum drawing temperature without material loss of red-hardness, or hardness at normal temperatures, and at the same time the distinctive properties of the alloy, including plasticity, strength, cutting efficiency and abrasion resistance, are maintained practically intact. Alloy A, for instance, as indicated in Table II, after heating at 1350° F., not only is almost as hard as when quenched but also has been endowed with the other properties mentioned, all of which are dependably preserved if the alloy is heated again for any purpose at any temperature up to about 1350° F. Especially in the respects noted in this paragraph, this invention appears to be entitled to be rated as a pioneer contribution to the art.

Some responses to thermal treatment manifested by alloys of this invention may seem analogous to similar responses that occur in high speed steel. My observation is, however, that the intermediate and resultant chemical compositions and physical structures of the new alloys are importantly different from those of high speed steel or other alloys of that general type, and that such differentials fully account for the unique stability against variation of pre-developed hardness through diffusion or atomic rearrangement at temperatures in excess of 1100° F., in contrast to the marked chemical and physical changes which occur above that temperature in heretofore known alloys of the high speed type. In the case of the present alloy the stability at and above 1100° F. results in a remarkably high degree of red-hardness in metal cutting tools. The expression "high degree of red-hardness" used herein and in the appended claims is to be understood as meaning that the alloy retains a high percentage of pre-developed hardness when temperatures up to approximately 1250° F. are generated in the working portion of a tool, and that the actual hardness in such portion of the alloy is sufficiently high to permit of efficient metal cutting for protracted periods.

My further observation is that boron or boron compounds are present at all times in each major

constituent of the new alloys and I believe that to be a major factor contributing to the superior properties of the alloys.

The expression "the remainder principally iron" when used in the appended claims is to be understood as meaning that, besides the recited alloy elements, the balance of the alloy is iron which may contain minor and not injuriously effective amounts of manganese, silicon and possibly other incidental impurities. It is to be understood further that the percentage of iron is in excess of the percentage of cobalt.

I claim as my invention:

1. An alloy comprising tungsten 12.00% to 20.00%, molybdenum 1.00% to 6.00%, cobalt 20.00% to 35.00%, boron 0.45% to 0.95%, carbon 0.35% to 0.85%, and the remainder principally iron, characterized by responsiveness to thermal treatment for the precise concurrent development of a predetermined hardness between 62 and 70 Rockwell C, a relatively high degree of red hardness, and stability against permanent variation of predeveloped hardness through diffusion or atomic rearrangement when subsequently heated to temperatures up to approximately 1275° F. for a period of time necessary to effect efficient brazing or other fabrication.

2. An alloy steel comprising the components named in claim 1, within the respective ranges stated, which is characterized by responsiveness to quench hardening and by the concurrent development, during thermal treatment, of inherent properties of high red hardness and stability against permanent material variation of pre-developed hardness when heated to a temperature substantially equivalent to the drawing temperature at which the pre-developed hardness was developed.

3. An alloy steel comprising the components named in claim 1, within the respective ranges stated, characterized by responsiveness to quench hardening and by the development of a relatively high degree of inherent red hardness through thermal treatment.

4. A heat-treated alloy steel for cutting-tools and the like comprising the components named in claim 1, within the respective ranges stated, characterized by stability against permanent material variation of pre-developed hardness when intermittently heated and cooled, in service, within a range of temperatures up to the maximum drawing temperature at which the pre-developed hardness was developed.

5. An alloy comprising the following components in approximately the percentages stated: tungsten 16.00%, molybdenum 4.00%, vanadium 1.00%, cobalt 30.00%, carbon 0.70%, boron 0.75%, and the remainder principally iron, characterized by responsiveness to quench hardening and by the concurrent development, during heat treatment, of inherent properties of high red hardness and stability against permanent material variation of pre-developed hardness when reheated to a temperature approximately the maximum drawing temperature at which the hardness was developed.

6. An alloy steel comprising the components named in claim 5 in approximately the percentages stated, characterized by responsiveness to thermal treatment for the concurrent development of inherent properties of high red hardness and stability against permanent material variation of pre-developed hardness when heated, in service, to temperatures within the range 800° F. to 1250° F.

7. An alloy steel comprising the components named in claim 5 in approximately the percentages stated, characterized by the development of hardness from approximately 69 to 65 Rockwell C when drawn at temperatures ranging from about 1200° F. to 1300° F. respectively, and by stability against permanent variation of the developed degree of hardness through diffusion or atomic rearrangement when subsequently heated to a temperature approximately equivalent to that of the maximum drawing temperature.

ANTHONY G. DE GOLYER.